

March 28, 1939.

H. D. HOLLER

2,151,764

PROCESS OF PURIFYING ANNEALING GASES

Filed Dec. 31, 1936



WITNESSES:

Wm. B. Sellers.  
James M. Ely

INVENTOR

Homer D. Holler.

By  
Ezra W. Savage  
ATTORNEY

## UNITED STATES PATENT OFFICE

2,151,764

PROCESS OF PURIFYING ANNEALING  
GASES

Homer D. Holler, Export, Pa., assignor to Westinghouse Electric & Manufacturing Company, East Pittsburgh, Pa., a corporation of Pennsylvania

Application December 31, 1936, Serial No. 118,553

2 Claims. (Cl. 148—16)

This invention relates to a process for purifying annealing gases.

In bright annealing stainless steel, it is necessary to remove the oxidizing impurities from the annealing gas to prevent oxidation of the surfaces of the steel.

In the processes employed heretofore in purifying an annealing gas, such as nitrogen, hydrogen or dissociated ammonia, the gas is usually subjected to the action of a dryer or desiccant to remove the water vapor and oxygen sometimes found in the gas. These processes have objectionable features, for example, it is not always possible to so purify the gas that it can be employed in bright annealing stainless steel without introducing oxidizing impurities, or the purifying elements employed are too expensive for general commercial use.

An object of this invention is the provision of a process for inexpensively purifying annealing gases.

Another object of this invention is to so purify an annealing gas selected from the group comprising nitrogen, hydrogen and mixtures thereof that it may be utilized in bright annealing stainless steel without introducing oxidizing impurities.

Other objects of this invention will become apparent from the following description when taken in conjunction with the accompanying drawing, the single figure of which is a view partly in section and partly in side elevation of apparatus suitable for practicing this invention.

Referring to the drawing, the apparatus for practicing this invention comprises a purifying apparatus 10 suitable for so purifying annealing gases, such as nitrogen, hydrogen and mixtures thereof, for example, dissociated ammonia, that the gases may be employed in bright annealing stainless steel without introducing oxidizing impurities. In practice, the apparatus 10 may be connected between some suitable source of annealing gas and an annealing chamber (not shown).

As illustrated in the drawing, the annealing gas may be supplied from any suitable source of supply, such as a storage tank 12. The flow of the annealing gas may be controlled by means of a valve 14 disposed in the pipe line 16 connecting the source of supply with the purifying apparatus. The apparatus comprises a substantially U-shaped container 18 having a cover plate 20 so fitted and secured thereto by means of bolts 22 as to make the purifying apparatus substantially air-tight. The legs of the U-shaped

container form chambers 24 and 26, the purpose of which will be explained hereinafter, while the bridge of the U-shaped container cooperates with the cover plate 20 to provide a constricted connecting passage 28 between the chambers 24 and 26. Packing glands 30 and 32 may be disposed in suitable openings in the cover plate 20 for receiving the connecting pipe line 16 from the source of supply 12 of the annealing gas and a supply pipe 34, respectively. The supply pipe 10 connects the chamber 26 of the purifying apparatus with an annealing chamber (not shown).

In practice, a metal 36, which upon heating will vaporize and react with oxidizing impurities in the annealing gas to form metallic oxides, is disposed in the chamber 24 of the U-shaped container. Metals which have been found suitable for such vaporization and reaction with the oxidizing impurities are zinc and cadmium.

In order to heat the metal 36 to a temperature 20 above its melting point to effect vaporization, a heater 38, which in the apparatus illustrated is an electrical heating element, is disposed to substantially enclose the lower end of the chamber 24. The heating element may be connected to 25 some suitable source of electrical supply (not shown). In order to regulate the heat supplied to the metal during the operation of the purifying apparatus, and to maintain the temperature 30 high enough to insure the vaporization of the metal, some suitable thermionic element (not shown) may be connected in the heater circuit and disposed to respond to predetermined temperatures of the metal 36 in the chamber 24 to control the operation of the heater 38. The heat 35 supplied to the metal 36 will depend upon the metal employed, since zinc has a melting point of about 419.4° C. and a boiling point of about 907° C., while cadmium has a melting point of 320.0° C. and a boiling point of about 767° C. 40

In operation the metal in the chamber 24 is heated to a selected temperature between its melting point and boiling point in order to evolve metallic vapors. An annealing gas, such as nitrogen, hydrogen or dissociated ammonia, is supplied 45 to the chamber from a suitable source of supply, such as the tank 12. When the annealing gas is admitted to the chamber 24, it contacts the metallic vapors and a reaction occurs between the metallic vapors and any oxidizing impurities, such 50 as water vapor or oxygen, which may be present in the annealing gas to form either zinc oxide or cadmium oxide depending upon the metal employed in the purifying apparatus.

After the oxidizing impurities have been re- 55

5 moved from the annealing gas, the purified gas flows through the constricted passage 28 into the cooling chamber 26 where it is cooled to approximately room temperature. The cooling of the  
10 gases in the chamber 26 may be effected by dissipating the heat from the chamber by radiation and convection or by some suitable refrigerating means (not shown). If there is an excess of metallic vapor in the chamber 24, the unreacted  
15 vapors may also flow through the constricted passage into the cooling chamber 26 where the unreacted vapors are condensed and solidified on the sides and bottom of the container, as illustrated at 40. The purified and cooled annealing  
15 gas in the chamber 26 is delivered directly to the annealing chamber (not shown) through the supply pipe 34.

20 Where it is desired to employ the process in a recirculating system, the gases from the annealing chamber should be partially purified by means of known dryers or desiccants before admission to the purifying apparatus. This is because the present process is more efficient in so purifying an annealing that it may be utilized in bright annealing stainless steel without introducing oxidizing impurities when most of the impurities have been removed by other means, such as the well known desiccants. By removing most of the impurities from annealing gases drawn directly  
25 from an annealing chamber prior to treating the gas by the present process, the metallic vapors utilized by this process to remove the oxidizing impurities are not contaminated with the large quantities of oxidizing impurities normally found  
30 in the furnace annealing gases.

35 The process of this invention is very efficient for removing the small quantities of oxidizing impurities found in annealing gases after they have been subjected to known purifying processes and the  
40 gases subjected to this process are suitable for bright annealing stainless steel. Further, since the metals zinc and cadmium are comparatively inexpensive and since the metallic oxide formed by the reaction between the metallic vapors and  
45 the small quantities of oxidizing impurities in the gas are readily reclaimed, an inexpensive process is provided for purifying the annealing gases, such

as nitrogen, hydrogen and dissociated ammonia. In addition to being inexpensive, the process may be easily controlled by controlling the temperature at which the metallic vapors are produced.

5 I claim as my invention:

1. A process of purifying an annealing gas to provide a non-oxidizing gas for bright annealing stainless steel comprising the steps of, heating a metal of the group consisting of zinc and cadmium in a substantially air-tight container at a 10 temperature of between the melting point and boiling point of the metal to vaporize it, delivering an annealing gas selected from the group consisting of nitrogen, hydrogen and dissociated ammonia into the metallic vapors whereby the metallic vapors react with the gas to remove oxidizing impurities from the gas, the reaction product of the metallic vapors and the oxidizing impurities being stable in each of nitrogen, hydrogen, and dissociated ammonia, providing for the flow 15 of the gas from the heating and reacting chamber into a cooling chamber wherein the gas and any metallic vapors carried therein are so cooled as to free the gas from the vapors by condensing them, and withdrawing the cooled and purified 25 gas from the cooling chamber.

2. A process of purifying an annealing gas to provide a non-oxidizing gas for bright annealing stainless steel comprising the steps of, heating zinc in a substantially air-tight container at a 30 temperature of between about 420° C. and about 907° C. to vaporize it, delivering an annealing gas selected from the group consisting of nitrogen, hydrogen and dissociated ammonia into the zinc vapors whereby the vapors react with the gas to 35 form vaporous zinc oxide thereby removing oxidizing impurities from the gas, the zinc oxide being stable in each of nitrogen, hydrogen and dissociated ammonia, providing for the flow of the gas from the heating and reacting chamber into 40 a cooling chamber wherein the gas and any zinc vapors carried therein are so cooled as to free the gas from the vapors by condensing them, and withdrawing the cooled and purified gas from the cooling chamber.

45 HOMER D. HOLLER.